# EUROPEAN PATENT SPECIFICATION

(11) **EP 0 518 510 B1**
(45) Date of publication and mention of the grant of the patent: **03.09.1997**
(21) Application number: 92304672.6
(22) Date of filing: 22.05.1992
(51) Int. Cl.: H01H 69/02, H01H 85/157

(54) **Electrical fuses**
Elektrische Schmelzsicherungen
Fusibles électriques

(30) Priority: 13.06.1991 GB 9112726
(43) Date of publication of application: 16.12.1992
(73) Proprietor: Cooper Industries Inc., Houston Texas 77002 (US)
(72) Inventor: Bacon, Martin David, Frome, Somerset BA11 1PP (GB); Drayton, Peter John, "The Cedars", Frome, Somerset BA11 4BB (GB); Peterson, Rognvald Ridley, Frome, Somerset BA11 2HT (GB)
(74) Representative: MacDougall, Donald Carmichael

(56) References cited:
- EP-A- 0 208 354
- EP-A- 0 334 473
- WO-A-90/00305

## Description

The present invention relates to miniature electrical fuses and more particularly to such fuses in which the fusible element is located within a tubular housing of an insulating material and connected between electrically conducting end caps which close off the opposite ends of the tubular housing and have electrical lead wires connected thereto to permit the fuse to be connected into a circuit without use of a fuse holder.

The invention is particularly concerned with problems arising from securing the electrical wires to the end caps in miniature fuses.

In known constructions the lead wires are generally welded or staked to external or secondary caps which are pushed on over the main end caps after manufacture of the main body of the fuse. This is because attempts to resistance weld lead wires directly to the main end caps give rise to a number of problems. Particular problems which occur are weakness of the lead attachment; distortion of the fusible element during welding which causes variation in the blowing characteristics of the fuse or loss of breaking capacity; and furthermore movement of solder fluidised during the welding process causes globules or streamers of solder to enter the fuse housing and affect the fuse performance.

W090/00305, on which the preambles of claims 1 and 6 are based, describes a microfuse comprising a fusible element bonded to a ceramic chip. The chip is contained within a tubular insulating enclosure having end caps to which the respective ends of the fusible element are coupled with solder. The solder also secures the ceramic chip to the end caps. Lead wires are attached to respective end caps.

It is an object of the present invention to provide a fuse construction and method of manufacture which is sufficiently robust to withstand the forces and thermal effects involved in resistance welding axial lead wires directly to the end caps of a fuse and on which the aforementioned problems are substantially reduced or avoided.

According to a first aspect of the present invention there is provided a method of manufacturing a miniature electrical fuse having a fusible element located within a tubular housing made of insulating material, the element being connected between electrically conducting end caps which close off the opposite ends of the housing, and the end caps having electrical lead wires connected thereto to permit the fuse to be connected into a circuit without use of a fuse holder, the method comprising the step of forming a sub-assembly by uniting the ends of the tubular housing and the fusible element to respective end caps of the tubular housing with a solder joint, characterised in that during said forming step an axial force is maintained on each end cap to urge each end cap into direct mechanical contact with the pertaining end face of the housing so that solder alloy is substantially absent from the site of said direct mechanical contact and in that, subsequent to the solder alloy having solidified, the method comprises the further step of simultaneously resistance welding the lead wires directly to respective end caps of the sub-assembly using opposed thrust forces which are transmitted through the said direct mechanical contacts to the tubular housing,

wherein the end caps are selected to have comparatively thick base portions and thin side walls, the thickness ratio being within the range 1.3 to 1 and 2.1 to 1, and the solder alloy is selected to have a comparatively high melting point, in excess of 180°C, whereby the sub-assembly is sufficiently robust to withstand the forces involved in the resistance welding process, the side walls of the end caps are sufficiently thin and elastic not to damage the housing when they contract in the solder cooling phase after the caps are soldered to the housing, the solder alloy is of sufficiently high melting point to prevent displacement of the fusible element or the solder joints of the sub-assembly during the resistance welding process, and the end faces of the housing are accurately plane parallel and orthogonal to the axis of the housing.

According to a second aspect of the present invention there is provided a miniature electrical fuse comprising a fusible element located within a tubular housing made of insulating material and connected between electrically conducting end caps which close off the opposite ends of the housing, the ends of the tubular housing and the fusible element being united to respective end caps by solder joints, and a pair of electrical lead wire secured to respective end caps, characterised in that the electrical lead wires are secured to respective end caps by resistance welded joints, the thickness of that part of the base of each end cap to which a lead wire is secured being greater than the thickness of the side wall of the cap in a ratio between 1.3 to 1 and 2.1 to 1, and in that the end caps are in direct mechanical contact with respective pertaining end faces of the tubular housing so that solder alloy is substantially absent from the sites of mechanical contact.

The invention will now be further described by way of example, with reference to the accompanying drawing which is an axial view partly in section and to an enlarged scale of one embodiment of fuse according to the invention.

Referring to the drawings, a fusible element comprising a helical wire 1 wound on an insulating support 2 is axially located in a cylindrical tubular glass housing 3 whose ends are closed off by electrically conducting metal end caps 4. the housing 3 could alternatively be made of ceramic or a filled plastic material and fusible element 1 could alternatively be a slant wire, an axial wire, or other element design known in the art. If desired the housing 3 may be filled with a suitable material e.g. quartz grains, ceramic particles, ceramic wool, ceramic cloth, ceramic paper, polymer granules, inorganic or organic materials intended to release arc-quenching substances when heated, or solid matrix ceramic materials.

The ends of the tubular housing 3 are made accurately plane parallel and perpendicular to the axis of the housing so that when the solder initially located within each end cap 4 is melted and the end cap is pushed on to the housing 3 during the assembly of the fuse, direct mechanical contact is achieved between the end cap and the end faces of the housing as shown at 5. In the case of a glass tube this accuracy of the tube end faces can be achieved by setting with a diamond wheel. In the case of a ceramic tube this can be achieved by end grinding after firing.

A flux is used initially to melt the solder into the caps 4 prior to assembly of the fuse, but after solder solidification and prior to such assembly the flux is removed by immersion in a solvent. This ensures that the assembled fuse has a solid metal joint between the end cap and the end faces of the tubular housing, without enclosures of solidified flux. Such enclosures of flux can lead to distortion of the fuse during the subsequent resistance welding process as the enclosures soften at comparatively low temperatures.

During the assembly process of the fuse when the solder is heated and the end caps 4 are pushed onto the housing 3, force is maintained on the ends caps 4 throughout the solder cooling process to ensure that the direct mechanical contact with the ends of the tubular housing is retained. The resulting solder joint between the housing 3 and the side wall of the end caps is shown at 6 and the solder joint to the fuse wire is shown at 7. Solder is substantially squeezed out from and therefore is effectively absent from the site 5 of direct mechanical contact between housing 3 and end caps 4.

To facilitate the subsequent resistance welding process after the solder has cooled and solidified, the solder is selected to have a comparatively high melting point (for example 180°C or greater) and preferably is an alloy of lead in the range 77-90% and tin in the range 23%-10%. One particular alloy which is suitable is 85% lead and 15% tin. Other alloys containing tin, lead, possibly with antimony and silver in varying proportions, may also be utilised.

Such an initial construction enables the fuse to withstand the forces and thermal effects involved in the subsequent resistance welding of the axial lead wires 8 directly to the end caps 4, the welds being shown at 9.

As can be seen, the base of each end cap 4 is thicker than the side wall of the cap within the ratio 1.3 to I and 2.1 to 1. The thick base of the end caps is provided to withstand the subsequent resistance welding process whereas the side wall of the end caps is comparatively thin and elastic so that during the solder cooling process the contraction of the side wall and solder joint 6 does not lead to excessive forces on the frangible side walls of the housing 3. For a fuse having a cylindrical tubular housing of approximately 5mm external diameter and an overall length of 15 to 24mm the thickness of the base of each end cap is typically 0.5 to 0.72mm and the side wall thickness is typically 0.3 to 0.45mm. The lead wires may be between 0.4 and 1.0mm in diameter and made of tin plated copper or tin plated copper clad steel.

To effect resistance welding of the lead wires 8 to the end caps 4 a clamp type electrode is simultaneously fitted to the side wall of each end cap 4 and each lead wire 8 is gripped by an electrode and urged axially into engagement with the pertaining end cap to form the welds 9. Thus the opposing axial forces from both lead wires 8 are transmitted by the comparatively thick end walls of the end caps 4 and their circumferential abutment with the end faces of the housing 3 to the housing itself. The thermal effects of the resistance welding process are greatest at the outermost surface of the end walls of the end caps 4 where the welds 9 are formed. Thus the thermal effects are comparatively remote from the solder joints 6,7 and because the solder is of high melting point it does not soften. The lead wires 8 are therefore simultaneously fitted directly to the end caps 4 without disturbing the pre-assembled main portion of the fuse.

It will be appreciated that various modifications may be made to the embodiment described above without departing from the scope of the invention as defined by the appended claims. For example only the central area of the base of each end cap to which the lead wire 8 is attached may be of increased thickness as indicated by the broken line configuration, 4a. Typically in this case the central portion to which the lead wire is welded may be of thickness between 0.5 and 1.0mm.

## Claims

1. A method of manufacturing a miniature electrical fuse having a fusible element (1) located within a tubular housing (3) made of insulating material, the element (1) being connected between electrically conducting end caps (4) which close off the opposite ends of the housing, and the end caps (4) having electrical lead wires (8) connected thereto to permit the fuse to be connected into a circuit without use of a fuse holder, the method comprising the step of forming a sub-assembly by uniting the ends of the tubular housing (3) and the fusible element (1) to respective end caps of the tubular housing (3) with a solder joint (6, 7), characterised in that during said forming step an axial force is maintained on each end cap (4) to urge each end cap (4) into direct mechanical contact with the pertaining end face of the housing (3) so that solder alloy is substantially absent from the site of said direct mechanical contact and in that, subsequent to the solder alloy having solidified, the method comprises the further step of simultaneously resistance welding the lead wires (8) directly to respective end caps (4) of the sub-assembly using opposed thrust forces which are transmitted through the said direct mechanical contacts to the tubular housing (3), wherein the end caps (4) are selected to have comparatively thick base portions and thin side walls, the thickness ratio being within the range 1.3 to 1 and 2.1 to 1, and the solder alloy is selected to have a comparatively high melting point, in excess of 180°C, whereby the sub-assembly is sufficiently robust to withstand the forces involved in the resistance welding process, the side walls of the end caps (4) are sufficiently thin and elastic not to damage the housing (3) when they contract in the solder cooling phase after the caps (4) are soldered to the housing, the solder alloy is of sufficiently high melting point to prevent displacement of the fusible -element (1) or the solder joints (6,7) of the sub-assembly during the resistance welding process, and the end faces of the housing (3) are accurately plane parallel and orthogonal to the axis of the housing (3).

2. The method claimed in claim 1, wherein prior to formation of said sub-assembly each end cap (4) is loaded with solder alloy in the presence of a flux and after solder solidification the flux is removed by immersion in a solvent to prevent inclusions of solidified flux in the solder joints of the sub-assembly.

3. The method claimed in claim 1 or claim 2, wherein the solder alloy is a composition of between 77% and 90% lead with the remainder being tin.

4. The method claimed in any preceding claim, wherein the tubular housing (3) is made of glass and the end faces are rendered accurately plane parallel and orthogonal to the axis of the housing (3) by cutting with a diamond wheel.

5. The method claimed in any one of claim 1 to 3, wherein the tubular housing (3) is made of ceramic and the end faces are reduced accurately plane parallel and orthogonal to the axis of the housing (3) by end grinding after firing.

6. A miniature electrical fuse comprising a fusible element (1) located within a tubular housing (3) made of insulating material and connected between electrically conducting end caps (4) which close off the opposite ends of the housing (3), the ends of the tubular housing (3) and the fusible element (1) being united to respective end caps (4) by solder joints (6,7), and a pair of electrical lead wires (8) secured to respective end caps (4), characterised in that the electrical lead wires (8) are secured to respective end caps by resistance welded joints (9), the thickness of that part of the base of each end cap (4) to which a lead wire (8) is secured being greater than the thickness of the side wall of the end cap (4) in a ratio between 1.3 to 1 and 2.1 to 1, and in that the end caps (4) are in direct mechanical contact with respective pertaining end faces of the tubular housing (3) so that solder alloy is substantially absent from the sites of mechanical contact.

## Patentansprüche

1. Verfahren zum Herstellen einer elektrischen Feinsicherung mit einem Schmelzelement (1), das sich in einem röhrenförmigen Gehäuse (3) befindet, das aus isolierendem Material besteht, wobei das Element (1) zwischen elektrisch leitende Abschlußkappen (4) geschaltet ist, die die einander gegenüberliegenden Enden des Gehäuses verschließen, und die Abschlußkappen (4) elektrische Zuleitungsdrähte (8) aufweisen, die daran angeschlossen sind, so daß die Sicherung ohne eine Sicherungsfassung in einen Stromkreis geschaltet werden kann, wobei das Verfahren das Herstellen einer Unterbaugruppe durch Verbinden der Enden des röhrenförmigen Gehäuses (3) und des Schmelzelementes (1) mit entsprechenden Abschlußkappen des röhrenförmigen Gehäuses (3) mittels einer Lötverbindung (6,7) umfaßt, **dadurch gekennzeichnet**, **daß** während des Herstellstellschrittes eine axiale Kraft auf jede Abschlußkappe (4) ausgeübt wird, um jede Abschlußkappe (4) in direkten mechanischen Kontakt mit der betreffenden Stirnfläche des Gehäuses (3) zu drücken, so daß an der Stelle des direkten mechanischen Kontaktes im wesentlichen keine Lötlegierung vorhanden ist, und dadurch, daß nach Verfestigung der Lötlegierung das Verfahren den weiteren Schritt des gleichzeitigen Widerstandsschweißens der Zuleitungsdrähte (8) direkt an entsprechende Abschlußkappen (4) der Unterbaugruppe unter Verwendung einander entgegengesetzter Schubkräfte umfaßt, die über die direkten mechanischen Kontakte auf das röhrenförmige Gehäuse (3) übertragen werden, wobei die Abschlußkappen (4) so ausgewählt werden, daß sie vergleichsweise dicke Basisabschnitte und dünne Seitenwände aufweisen, wobei das Dickenverhältnis im Bereich zwischen 1,3 zu 1 und 2,1 zu 1 liegt und die Lötlegierung so ausgewählt wird, daß sie einen vergleichsweise hohen Schmelzpunkt von über 180°C, aufweist, so daß die Unterbaugruppe robust genug ist, um den Kräften zu widerstehen, die beim Widerstandsschweißvorgang auftreten, die Seitenwände der Abschlußkappen (4) ausreichend dünn und elastisch sind, um das Gehäuse (3) nicht zu beschädigen, wenn sie sich bei der Lötabkühlphase zusammenziehen, nachdem die Kappen (4) an dem Gehäuse angelötet wurden, die Lötlegierung einen ausreichend hohen Schmelzpunkt aufweist, um Verschiebung des Schmelzelementes (1) oder der Lötverbindungen (6,7) der Unterbaugruppe während des Widerstandsschweißvorgangs zu verhindern, und die Stirnflächen des Gehäuses (3) genau planparallel und rechtwinklig zur Achse des Gehäuses (3) sind.

2. Verfahren nach Anspruch 1, wobei vor der Herstellung der Unterbaugruppe jede Abschlußkappe (4) beim Vorhandensein eines Flußmittels mit Lötlegierung gefüllt wird, und nach der Lötverfestigung das Flußmittel durch Eintauchen in ein Lösungsmittel entfernt wird, um Einschlüsse von verfestigtem Flußmittel in den Lötverbindungen der Unterbaugruppe zu verhindern.

3. Verfahren nach Anspruch 1 oder Anspruch 2, wobei die Lötlegierung eine Zusammensetzung aus 77 % bis 90 % Blei ist, wobei der Rest Zinn ist.

4. Verfahren nach einem der vorangehenden Ansprüche, wobei das röhrenförmige Gehäuse (3) aus Glas besteht und die Stirnflächen genau planparallel und rechtwinklig zur Achse des Gehäuses (3) ausgeführt werden, indem sie mit einer Diamantscheibe geschnitten werden.

5. Verfahren nach einem der Ansprüche 1 bis 3, wobei das röhrenförmige Gehäuse (3) aus Keramik besteht und die Stirnflächen nach dem Brennen durch Stirnschweißen genau planparallel und senkrecht zur Achse des Gehäuses (3) verringert werden.

6. Elektrische Feinsicherung, die ein Schmelzelement (1) umfaßt, das sich in einem röhrenförmigen Gehäuse (3) befindet, das aus isolierendem Material besteht, und das zwischen elektrisch leitende Abschlußkappen (4) geschaltet ist, die die einander gegenüberliegenden Enden des Gehäuses (3) verschließen, wobei die Enden des röhrenförmigen Gehäuses (3) und des Schmelzelementes (1) mit entsprechenden Abschlußkappen (4) mittels Lötverbindungen (6,7) verbunden sind, sowie ein Paar elektrischer Zuführungsdrähte (8), die an entsprechenden Abschlußkappen (4) befestigt sind, **dadurch gekennzeichnet, daß** die elektrischen Zuleitungsdrähte (8) an entsprechenden Abschlußkappen mittels widerstandsgeschweißter Verbindungen (9) befestigt sind, wobei die Dicke des Teils der Basis jeder Abschlußkappe (4), an der ein Zuleitungsdraht (8) befestigt ist, in einem Verhältnis zwischen 1,3 zu 1 und 2,1 zu 1 größer ist als die Dicke der Seitenwand der Abschlußkappe (4), und daß die Abschlußkappen (4) in direktem mechanischen Kontakt mit entsprechenden betreffenden Abschlußflächen des röhrenförmigen Gehäuses (3) sind, so daß an den Stellen mechanischen Kontakts im wesentlichen keine Lötlegierung vorhanden ist.

## Revendications

1. Procédé de fabrication d'un fusible électrique miniature comportant un élément fusible (1) situé à l'intérieur d'un boîtier (3) tubulaire réalisé en matériau isolant, l'élément (1) étant connecté entre des capots (4) d'extrémité électriquement conducteur qui ferment les extrémités opposées du boîtier, les capots d'extrémité (4) ayant des câbles (8) de conducteur électrique connectés à ceux-ci pour permettre au fusible d'être connecté dans un circuit sans l'utilisation d'un support de fusible, le procédé comprenant les étapes consistant à former un sous-ensemble en unissant les extrémités du boîtier tubulaire (3) et l'élément fusible (1) aux capots d'extrémité respectifs du boîtier tubulaire (3) avec un joint de soudure (6,7), caractérisé en ce qu'au cours de ladite étape de formation, une force axiale est maintenue sur chacun des capots d'extrémité (4) pour solliciter chacun des capots d'extrémité (4) en contact mécanique direct avec la face d'extrémité correspondante du boîtier (3) de sorte qu'un alliage de soudage est sensiblement absent de la zone dudit contact mécanique direct et en ce que, après la solidification de l'alliage de soudage, le procédé comporte en outre l'étape de soudage électrique par résistance simultanée des câbles conducteurs (8) directement sur les capots d'extrémité (4) respectifs du sous-ensemble utilisant des forces de poussée opposées qui sont transmises à travers lesdits contacts mécaniques directs au boîtier tubulaire (3), dans lequel les capots d'extrémité (4) sont choisis pour avoir des parties de base d'épaisseur comparable et des parois d'extrémité minces, le rapport d'épaisseur se situant dans la gamme allant de 1,3 à 1 et de 2,1 à 1, et l'alliage de soudage étant sélectionné pour avoir un point de fusion comparativement haut, d'au moins 180°C, de sorte que le sous-ensemble est suffisamment robuste pour supporter les efforts impliqués au cours du procédé de soudage électrique par résistance, les parois latérales des capots d'extrémité (4) étant suffisamment minces et élastiques pour ne pas endommager le boîtier (3), lorsqu'ils se contractent dans la phase de refroidissement de la soudure après que les capots (4) aient été soudés au boîtier, l'alliage de soudage ayant un point de fusion suffisamment haut pour prévenir un déplacement de l'élément fusible (1) ou des joints de soudage (6,7) du sous-ensemble, au cours du procédé de soudage électrique par résistance, et une face d'extrémité du boîtier (3) étant précisément plane, parallèle et perpendiculaire à l'axe du boîtier (3).

2. Procédé selon la revendication 1, dans lequel avant la formation du sous-ensemble, chaque capot d'extrémité (4) est chargé avec un alliage de soudage en présence d'un flux et après solidification de la soudure, le flux est enlevé par immersion dans un solvant pour prévenir des inclusions de flux solidifié dans les joints de soudure du sous-ensemble.

3. Procédé selon l'une des revendications 1 et 2, dans lequel l'alliage de soudage est une composition comportant entre 77% et 97% de plomb, le reste étant constitué d'étain.

4. Procédé selon l'une quelconque des revendications précédentes, dans lequel le boîtier tubulaire (3) est réalisé en verre et les faces d'extrémité sont rendues précisément planes, parallèles et perpendiculaires à l'axe du boîtier (3), par découpage avec une roue de diamant.

5. Procédé selon l'une quelconque des revendications 1 à 3, dans lequel le boîtier tubulaire (3) est réalisé en céramique et les faces d'extrémité sont rendues précisément planes, parallèles et perpendiculaires à l'axe du boîtier (3) par ponçage après cuisson.

6. Fusible électrique miniature comprenant un élément fusible (1) situé dans un boîtier tubulaire (3) réalisé en un matériau isolant et connecté entre des capots (4) d'extrémité électriquement conducteurs qui ferment les extrémités opposées du boîtier (3), les extrémités du boîtier tubulaire (3) et l'élément fusible (1) étant unis aux capots d'extrémité (4) par des joints de soudure (6,7), et une paire de câbles conducteurs électriques (8) fixés aux capots (4) d'extrémité respectifs, caractérisé en ce que les câbles (8) conducteurs électriques sont fixés aux capots d'extrémité respectifs par des joints (9) soudés par résistance électrique, l'épaisseur de cette partie de la base de chaque capot d'extrémité (4) à laquelle le câble (8) conducteur est fixé étant supérieure à l'épaisseur de la paroi latérale du capot d'extrémité (4) dans un rapport se situant entre 1,3 à 1 et 2,1 à 1, et en ce que les capots (4) d'extrémité sont en contact mécanique direct par rapport aux faces d'extrémité correspondantes du boîtier tubulaire (3) de sorte qu'un alliage de soudage est sensiblement absent des zones de contact mécanique.
